

Jan. 25, 1927.

1,615,707

C. E. JONES ET AL

CORROSION RESISTING METAL

Filed Nov. 10, 1924



COATED WITH CADMIUM AND TIN

Inventors:

Charles E. Jones,  
Mark A. Atuesta,

by *Mark A. Atuesta*,  
Their Attorney.

Patented Jan. 25, 1927.

1,615,707

## UNITED STATES PATENT OFFICE.

CHARLES E. JONES AND MARK A. ATUESTA, OF SCHENECTADY, NEW YORK, ASSIGNEES TO GENERAL ELECTRIC COMPANY, A CORPORATION OF NEW YORK.

### CORROSION-RESISTING METAL.

Application filed November 10, 1924. Serial No. 748,941.

Our present invention relates particularly to the protection against corrosion of iron and steel, but may be applicable to other metals as well.

5 Iron and steel are often used in places where the metal is not only subject to ordinary atmospheric corrosion or rusting, but also to more active chemical action by fumes or corrosive liquids. Under the combined 10 action of these deteriorating agencies, the life of articles made of ferrous metal is likely to be very short. Ordinary rust-proofing treatment will effect but little improvement as the coating agents used for 15 rust-proofing usually will not withstand the corrosion caused by acid fumes or the like.

In accordance with our invention we have provided a composite coating which will withstand both the conditions leading to 20 rusting and also acidic corrosion. This coating comprises a layer of a rust-proofing metal, such for example as cadmium, overlaid by a layer of a metal capable of withstanding acids, as tin, for example.

25 A practical utilization of our invention is illustrated by the accompanying drawing, which shows in perspective a trolley wire hanger as an example of an object coated in accordance with our invention with the 30 above attendant advantages.

In carrying out our invention the metal article is cleaned by the usual well known method to produce a surface condition suitable for electroplating. A film of cadmium 35 may be applied by any well known method. For example, a plating bath comprising a solution in water of a cadmium salt, a cyanide and an alkali may be used. We have used the following solution with success 40 with a current density of about 8 to 10 amperes per square foot:

Cadmium hydrate, 4 ounces; sodium cyanide, 6 ounces; caustic soda, 1 ounce; water, 1 gallon.

45 The thickness of the cadmium film, of course, may be varied with conditions. We have found that a coating of about one mil in thickness produced by plating at the above current density for about thirty 50 minutes at room temperature is sufficient.

A tin film may be applied by any ap-

proved method. For example a solution of the following composition may be used:

Tin chloride, 2 ounces; sodium cyanide, 1/2 ounce; caustic soda, 8 ounces; cream of 55 tartar, 1 ounce; water, 1 gallon.

With a current density of ten amperes per square foot a suitable coating may be deposited from the above bath in about fifteen minutes at room temperature.

50 The electrolytic potential of tin with respect to a ferrous metal is so considerable that a ferrous metal article coated with tin alone would be attacked very rapidly in the presence of an electrolyte such as water containing an acid wherever the tin coating was locally imperfect due to wear, or an accidental scratch or any other reason. The presence of the cadmium however will protect the ferrous metal even when the tin 70 coating is marred. On the other hand, cadmium alone will not withstand as well as tin the influence of acidic corrosion.

55 Some of the benefits of our invention may be obtained by using zinc as the rust-proofing metal in place of cadmium and thereupon applying tin over the zinc coating, and we desire the appended claims, therefore, to include zinc as equivalent to cadmium.

We have shown for illustration a trolley 60 wire hanger provided with successive coatings of cadmium or zinc and tin. A hanger thus coated is well adapted to withstand the severe conditions existing in mines where the conditions tend to produce rapid corrosion 65 of the metal. Other applications will suggest themselves. Our invention is of value for rust-proofing of steel clamps used for holding leather during the process of treatment, particularly when making the so-called 70 "patent leather".

75 What we claim as new and desire to secure by Letters Patent of the United States, is:

An article of manufacture comprising a 80 body of ferrous metal, a film of cadmium thereon and a film of tin overlaying said cadmium film.

In witness whereof, we have hereunto set our hands this 7th day of November, 1924.

CHARLES E. JONES.  
MARK A. ATUESTA.